

## UNITED STATES PATENT OFFICE

2,642,375

## HEMOSTATIC COMPOSITIONS

John Henderson, New Market, and Alfred Bloch and Herbert L. Davis, Highland Park, N. J., assignors to Ethicon Suture Laboratories Incorporated, a corporation of New Jersey

No Drawing. Application August 21, 1951,  
Serial No. 242,992

3 Claims. (Cl. 167—65)

1

This invention relates to new and improved hemostatic compositions and specifically relates to such compositions that are absorbable in body fluids by physiologic processes.

Various substances and compositions have been employed by members of the medical profession to control bleeding of soft tissues and cut bone surfaces. Natural clotting agents such as striated muscle have been used, particularly in neurosurgery and in drill holes in bone. Certain plasma fractions have been used, and fibrin from whipped blood has been so prepared that it could be immediately plastered on bleeding surfaces. Human fibrin foam has been used as a carrier of thrombin, and the fibrin foam has been used in the form of a dry, porous, brittle, cream-colored textile. Another plasma protein, thrombin, in a highly potent, purified, water-soluble form has been used as a hemostatic spray as well as in conjunction with human fibrin foam, but thrombin is unstable in aqueous solution and cannot be heat sterilized in an autoclave without destroying its activity as a hemostatic substance. Fibrinogen in conjunction with thrombin has also been found useful in the formation of an adhesive layer to seal together cut surfaces of soft tissues, notably a skin graft on a prepared bed. More recently an absorbable substance in the form of a sponge has been used and is prepared from a specially prepared gelatin solution which is further processed and sterilized. The gelatin sponge when dry is a light, off-white, reasonably tough, porous substance that may be readily cut by a sharp instrument into any desired shape or size. This absorbable gelatin sponge is normally used in conjunction with a thrombin solution. The gelatin sponge mixed with the thrombin solution is used by applying it to a bleeding area where it quickly imbibes blood which clots as it comes in contact with thrombin. Physiological absorption of the sponge takes place in from 15 to 20 days.

Another recent absorbable substance which has found acceptance by the medical profession as a hemostatic agent is oxidized cellulose. It was found that oxidized cellulose in the form of cotton, paper, gauze, or a non-woven mass had hemostatic properties, and its use as a hemostatic agent has been widely studied in a variety of animal and human tissues. The material was demonstrated to be non-irritating and to disappear in the tissue leaving a minimum of scar.

The control of osseous hemorrhage has presented a serious problem to the medical profession because the hemostatic agents found effective for the control of soft tissue hemorrhages

2

have not been effective for the control of bleeding from cut bone surfaces. One class of materials used for the control of this latter type of hemorrhage is called bone wax. Bone waxes in common use today are prepared from refined waxes of bees which have been admixed with other non-absorbable and water-insoluble hydrocarbons or vegetable oils. Bone wax has been used for the purpose of controlling hemorrhages from the cut surfaces of bones, such as those of the skull, by forcibly smearing the wax over the cut surface so that the material acts mechanically to occlude and seal the open ends of bleeding osseous vessels and sinuses. Such compositions have no specific hemostatic effect per se and quite often result in delayed healing because of their non-absorbable properties. Non-absorbable bone waxes, since they are left in the wound as a foreign body, frequently constitute a troublesome barrier to subsequent osseous union. Another disadvantage of non-absorbable bone wax is the danger of particles of the wax falling off the bone edge and lodging in the surrounding tissue where they provide a foreign body response which retards healing and may result in an inflammatory tissue response.

It is an object of this invention to prepare a hemostatic composition which is completely absorbable by body tissues.

It is another object of this invention to prepare a hemostatic composition which quickly controls hemorrhages from the cut surfaces of soft tissues and more particularly bones.

It is another and further object of this invention to prepare an absorbable hemostatic composition which possesses a specific hemostatic effect and is at the same time absorbable by physiologic processes.

It is still another and further object of this invention to prepare an absorbable hemostatic composition which is readily sterilizable by ordinary autoclaving procedures.

Other objects will be apparent from the following description and examples.

In accordance with the present invention it has been found that hemostatic compositions which have a specific hemostatic effect and in which the range of consistency varies from a highly viscous liquid to that of a soft wax and from a soft wax to that of a semi-solid or solid may be prepared which include as ingredients a water-soluble innocuous base and a hemostatic agent. The base may be a single substance or a mixture of two or more water-soluble innocuous substances, and the hemostatic agent is prefer-

ably a single substance, but a combination of hemostatic agents may be used.

Substances found suitable as bases include polymerized low molecular weight aliphatic glycols such as polymerized ethylene glycol, and low molecular weight ethers or esters of polyglycols such as the methyl, ethyl or propyl ethers of polyethylene glycols and the acetic or propionic esters of polyethylene or polypropylene glycols. Polymerized ethylene glycol is the preferred water-soluble base, and polymerized ethylene glycols having a molecular weight of from 200 to 4000 and a consistency varying from a liquid of low viscosity to that of a solid wax have been used. A combination of two or more polymerized ethylene glycols having molecular weights within this range may also be used, and for the preparation of bone wax it has been found preferable to use a polymerized ethylene glycol having a molecular weight of 1000 to 4000 in combination with a polymerized ethylene glycol having a molecular weight of from 200 to 600.

Hemostatic agents which have been found valuable for use in combination with a water-soluble innocuous base include oxidized cellulose, pectic acid, alginic acid and its salts including its calcium salts as well as a nitrated calcium salt of alginic acid and other alginic acid derivatives.

The preferred absorbable hemostatic agent for use in combination with a water-soluble innocuous base is oxidized cellulose. The oxidized cellulose which is used is that which results from the oxidation of cellulose with nitrogen dioxide as disclosed in U. S. Patent No. 2,232,990, issued February 25, 1941, and in the Journal of the American Chemical Society, volume 64, page 121, 1942, and whose properties are disclosed in the Journal of the American Chemical Society, volume 64, page 127, 1942. Such an oxidized cellulose is described as a homogeneous, alkali-soluble, non-nitrated, undegraded cellulose. The oxidation is disclosed as being accomplished by the use of gaseous nitrogen dioxide on cotton which results in the oxidation of the terminal carbon atoms of the glucose units of cellulose with the resultant formation of carboxyl groups at the said terminal carbon atoms. Oxidized cellulose prepared by this method exhibits a carbon dioxide equivalency of at least 15% and a complete solubility in aqueous sodium hydroxide in 2% concentration. It has been shown that oxidized cellulose having the above physical properties is completely absorbable by body tissues and that tissue slices utilize such oxidized cellulose as a nutrient substrate.

The preferred hemostatic formulation includes as ingredients polymerized ethylene glycol and oxidized cellulose. The oxidized cellulose is in the form of particles in the shape of rods which have an average diameter of 4 to 8 microns and an average length of 10 to 25 microns; the preferred average length is 15 to 20 microns.

In compounding oxidized cellulose with polymerized ethylene glycol the former is added to the latter at a temperature below 100° C., and the addition is made while the polymerized ethylene glycol is being efficiently stirred. It is preferred that the polymerized ethylene glycol base be a mixture of two or more polymerized ethylene glycol compounds of different molecular weights; one having a molecular weight between 1000 and 4000 which has a wax-like consistency and one having a molecular weight of less than 200 to 600 which is liquid in consistency. In preparing a bone wax in which two polymerized

ethylene glycol compounds are used, the two are mixed and heated and a uniform melt is obtained with the temperature of the melt preferably not above 100° C. The melt is allowed to cool to a temperature below 100° C. and pulverized oxidized cellulose is then added while the whole is being stirred efficiently, and stirring is continued until the mass is in a semi-solid state in order that separation and sedimentation of the oxidized cellulose particles will not occur.

The following examples of compositions, in which the parts are given by weight, comprising physical mixtures of polymerized ethylene glycol and oxidized cellulose, have been found suitable for use as a bone wax.

*Example I*

|                                                                     |    |
|---------------------------------------------------------------------|----|
| Polymerized ethylene glycol having average molecular weight of 1540 | 60 |
| Polymerized ethylene glycol having average molecular weight of 300  | 10 |
| Oxidized cellulose                                                  | 30 |

*Example II*

|                                                                        |    |
|------------------------------------------------------------------------|----|
| Polymerized ethylene glycol having an average molecular weight of 4000 | 35 |
| Polymerized ethylene glycol having an average molecular weight of 200  | 35 |
| Oxidized cellulose                                                     | 30 |

Formulations may be prepared which are satisfactory as hemostatic agents for use in connection with hemorrhages of soft tissues and bone hemorrhages in which the base consists of a single polymerized ethylene glycol which has a molecular weight as high as 1500; but when a polymerized ethylene glycol is used which has a molecular weight higher than 1500, some low molecular weight polymerized ethylene glycol must be added as a softening agent. The low molecular weight liquid portion of the polymerized ethylene glycol base may be present in an amount as high as 40% or 50% by weight if a high molecular weight polymerized ethylene glycol is used which has a molecular weight of from three to four thousand. By increasing the liquid polymerized ethylene glycol constituent, the formulations are made softer; and by increasing this ingredient still further, hemostatic compositions having a cream-like consistency are produced. A hemostatic formulation specifically for use on cut bone surfaces is preferred to have a semi-solid consistency such that it can be kneaded between the fingers when at room temperature.

The hemostatic action of a therapeutic composition prepared according to the preceding examples depends upon the presence of both the polymerized ethylene glycol constituent or constituents and powdered oxidized cellulose, since either of the compounds when used alone is not a satisfactory hemostatic agent, when applied to cut bone surfaces. Oxidized cellulose in powdered form when used alone does not adhere to bleeding cut surfaces of soft tissue or bone. Oxidized cellulose of itself has hemostatic properties, and the polymerized ethylene glycol with which it is intimately admixed and which is absorbable in body fluids enhances the hemostatic action of the oxidized cellulose by enabling it to come in close physical contact and actually to penetrate into severed blood vessels at the surface of cut soft tissues and into severed blood vessels and sinuses present on cut bone surfaces. The finely divided particles of oxidized cellulose which are then present at the openings and inside of blood

vessels and sinuses exert their hemostatic properties and effectively control bleeding.

Chemical reactions of the clotting mechanism of blood are set up when blood contacts oxidized cellulose due to the hemostatic properties of oxidized cellulose. Oxidized cellulose combines chemically with the hemoglobin of the blood and forms a large molecule which agglutinates into a gelatinous mass which in turn acts mechanically to stop the flow of blood in the same way as a true blood clot. In order for oxidized cellulose to stop bleeding it must be in firm contact with blood for about two minutes since this amount of time is necessary for the process described above to proceed to a point where the agglutinated substance can act mechanically to stop bleeding. The polymerized ethylene glycol of the composition, because of its water-soluble properties, enables oxidized cellulose to remain in contact with blood issuing from the vessels of cut soft tissue and bone surfaces long enough for the above chemical reaction to occur.

In order for a clot to be effective in stemming the flow of blood from a blood vessel or capillary, a clot must be produced inside a severed blood vessel since a clot on the surface of cut soft tissue or bone is readily and quickly removed from the site by the pressure of blood issuing from severed vessels. The intimate association of a water-absorbable base such as polymerized ethylene glycol with a finely divided hemostatic agent such as oxidized cellulose enables the particles of oxidized cellulose to enter blood vessels at their severed ends when such a composition is smeared or rubbed over cut surfaces of soft tissue and bones because the polymerized ethylene glycol dissolves in blood and penetrates into blood vessels and in doing so carries with it particles of oxidized cellulose.

Since certain changes may be made in the proportions of the ingredients composing the hemostatic therapeutic composition, and since certain ingredients may be varied without departing from the scope of the invention, it is intended that all matter contained in the above description shall be interpreted as illustrative and not in a limiting sense, but that the invention is to be limited only by the scope of the appended claims.

What is claimed is:

1. A hemostatic composition for use in the control of tissue and osseous hemorrhage com-

prising; as a water-soluble innocuous base, polymerized ethylene glycol having an average molecular weight of approximately 1500; and, as a hemostatic agent, finely divided oxidized cellulose intimately admixed therewith.

2. A hemostatic composition for use in the control of tissue and osseous hemorrhage comprising; as a water-soluble innocuous base, a mixture of a polymerized ethylene glycol having an average molecular weight of from 200 to 600 and a polymerized ethylene glycol having an average molecular weight of from 1000 to 4000; and, as a hemostatic agent, finely divided oxidized cellulose intimately admixed therewith.

3. A hemostatic composition for use in the control of tissue and osseous hemorrhage comprising; as a water-soluble innocuous base, a mixture of approximately 60 parts by weight of a polymerized ethylene glycol having an average molecular weight of approximately 1540 and 10 parts by weight of a polymerized ethylene glycol having an average molecular weight of approximately 300; and, as a hemostatic agent, 30 parts by weight of finely divided oxidized cellulose with particles in the shape of rods having an average diameter of 4 to 8 microns and an average length of 10 to 25 microns intimately admixed therewith.

JOHN HENDERSON.  
ALFRED BLOCH.  
HERBERT L. DAVIS.

References Cited in the file of this patent

UNITED STATES PATENTS

| Number    | Name    | Date          |
|-----------|---------|---------------|
| 2,160,503 | Hermann | May 30, 1939  |
| 2,185,255 | Kroper  | Jan. 2, 1940  |
| 2,558,395 | Studer  | June 26, 1951 |

FOREIGN PATENTS

| Number  | Country | Date          |
|---------|---------|---------------|
| 705,450 | Germany | Apr. 29, 1941 |

OTHER REFERENCES

- 45 Seegers et al., Hemostatic Agents, C. C. Thomas, Springfield, Illinois, 1948, pages 45, 90.  
McClelland et al., Chemical and Engineering News, February 10, 1945, volume 23, Number 3, pages 247, 250.

- 50 Anderson Squibb Abstract Bulletin, volume 18, page 1369 (1945).